

Jan. 16, 1951

M. S. HUDSON

2,538,457

TREATING WOOD

Filed Nov. 2, 1946



Inventor

*Monie S. Hudson*

By *Harley L. Parrott*

Attorney

## UNITED STATES PATENT OFFICE

2,538,457

## TREATING WOOD

Monie S. Hudson, Spartanburg, S. C.

Application November 2, 1946, Serial No. 707,489

8 Claims. (Cl. 260—124)

1

This is a continuation-in-part of my copending application Serial No. 457,236, filed September 3, 1942, now abandoned.

This invention relates to the processing of wood for hydrolyzing the same and the production of an improved completely dried hydrolyzed wood. The product is characterized by being substantially devoid of water soluble extractives produced by acid hydrolysis and further substantially devoid of organic solvent soluble extractives, either normally present or produced by the hydrolysis. Such a completely dried product has numerous advantages, among which may be mentioned the ease with which a potentially reactive resin may be incorporated in the same and the stability of the wood product when exposed to moisture.

The primary object of the invention is the provision of an improved rapid, economical and reliable process for producing such a completely dried hydrolyzed wood in massive or comminuted form, or in the form of powder or flour suitable for molding purposes. This process employs (1) hydrolyzing during which condensates from the steam and products of the hydrolysis reaction soluble therein are constantly removed from contact with the wood and from the treating chamber, and (2) the drying of such hydrolyzed wood in an atmosphere of an organic drying medium which is a solvent for organic solvent soluble extractives produced by the hydrolysis or already present in the wood whereby the same are removed from the wood. In other words, the process assures that the condensates from steam and hydrolysis products soluble therein are continually removed during hydrolysis whereby such valuable by-products may be recovered in a form free from degradation and that objectionable organic solvent soluble extractives produced by hydrolysis or already present are simultaneously removed in the drying operation incident to forming wood having a zero moisture content.

In the manufacture of hydrolyzed products in accordance with the invention from wood in the form of structural lumber, plywood and comminuted wood and similar materials, the same is subjected to a vapor treatment with either steam containing small amounts of hydrochloric acid, as a catalyst, or steam with small amounts of aniline to produce mild hydrolysis for the purpose of removing hemicelluloses. After this vapor treatment, pressure with air or inert gas may be built up in the wood in the treating chamber. The treating chamber is then filled with water still maintaining the pressure of inert gas

2

or air, as in the Rueping process (see United States Patent No. 709,799, Reissue No. 12,707, and Patent No. 1,008,864). Water is driven into the wood by employing a higher pressure, and this water serves to wash out the hydrolysis products on the release of the pressure and institution of vacuum or suitable reduced pressure conditions. One or more of these cycles may be employed for completely washing out the hydrolysis products from the wood. The wood may then be dried by employing vapor phase drying, as described in my Patent No. 2,273,039 and my application Serial No. 579,851, now Patent No. 2,435,218, using a suitable drying medium such as Stoddard solvent. As disclosed in my above identified patents, in effecting dehydration of wood any suitable organic material which can be vaporized and which vapor will permeate wet wood and flash off the moisture content thereof without deleteriously affecting the wood may be used. There are numerous and practically unlimited examples of suitable materials, but representative examples of satisfactory materials are as follows:

25 25. Organic compounds, whether saturated or unsaturated, chain or cyclic, and any of their homologues that might be suitable for this procedure, such as alcohols, ethers, amines, acids, aldehydes, ketones, esters, halides, cyanides, sulphides, polyhydric alcohols, anhydrides such as phthalic and nitro compounds; of which the following are examples:

n-Decane  
35 n-Decyl alcohols  
n-Decyl ethers  
n-Decyl amines  
n-Decyl esters  
n-Decyl halides  
40 n-Decanoic acids  
n-Decyl ketones  
n-Decyl aldehydes  
n-Decyl cyanides  
n-Decyl sulphides

45 50 Preferred examples of suitable organic drying mediums are creosote, petroleum distillates, coal tar, wood tar or wood distillates, and the following:

50 55 Aromatic hydroxy compounds:

Phenols  
Cresols  
Xylenols

55 56 High boiling acids—Oleic

## High boiling alcohols:

Amyl  
Isopropyl  
Isobutyl  
Diethylene glycol  
Glycerol

## Aldehydes:

Butyric aldehyde  
Benzaldehyde  
Crotonaldehyde  
Furfural

## High boiling amines:

Aniline  
Dimethyl-aniline  
Mono-, di- and tri-ethanolamines  
Pyridines  
Quinolines

## High boiling esters:

Butyl acetate  
Amyl acetate  
Butyl lactate  
Dibutylphthalate  
Diamylphthalate  
Glycol monoethyl ether acetate  
Isopropyl lactate  
Octyl acetate  
Diglycololeate  
Glycol stearate

## High boiling ethers:

Diamyl ether  
Diethylene glycol monoethyl ether

## Halides:

Chlorobenzenes  
Chlorinated phenols  
Nitrochlorobenzenes  
Ortho-dichlorobenzenes  
Ortho-nitrochlorobenzenes  
Para-dichlorobenzenes

## Nitro compounds:

Nitrobenzene  
Ortho-nitrotoluenes

## Hydrocarbons:

Benzenes  
Toluenes  
Mesitylenes  
Cumenes  
Naphthalenes  
Diphenyl

## Ketones—Benzophenone

Furfural or other resin forming material may be used as the drying medium if it is desired to leave in the wood resinous condensation products, i. e., to incorporate a synthetic resin in the wood.

In the manufacture of hydrolyzed products, by means of acid hydrolysis, in accordance with this invention, from comminuted wood the material is wetted with a solution of a mineral acid, e. g., sulfuric acid of about 1% strength and subjected in a rotating basket in a closed cylinder to the action of steam at a temperature of 340 to 360° F. (105 to 135 lbs./sq. in. gauge pressure) for a period of 20 to 40 minutes, depending on the particle size of the comminuted wood and the lignin content desired in the final product. The steam pressure is then released through a line in the bottom of the treating cylinder so that condensates and drainings from the wood, which contain sugars, furfural, and other by-products are forced into a condensate flash tank in which there is a line in the vapor space leading to the atmosphere. By releasing the pressure in the flash tank to the atmosphere the hydrolysis liquor containing sugars and non-volatile substances is concentrated. The steam being released is lead through suitable heat exchangers

both for the purpose of recovering heat and steam volatile by-products such as furfural and acetic acid by condensation.

When the pressure in the cylinder has reached atmospheric, wash water may be introduced and the hydrolyzed wood product washed by rotating the basket. After each washing period the wash water is drained off and a spray of wash water directed on the rotating basket from a spray line provided in the cylinder. Washings in the manner described are continued until the hydrolyzed product is free of hydrolyzing acid and products of hydrolysis. A satisfactory indication of this point is when a distilled water sample in which 15 a sample of the hydrolyzed wood has been boiled shows a pH of 5.0 to 6.0.

The washed hydrolyzed product may then be vapor dried in the same cylinder by subjecting it to the action of the vapor from a boiling hydrocarbon, such as Stoddard solvent, or other suitable organic drying or drying and impregnating medium, introduced to the cylinder while rotating the basket. The solvent may be removed if desired after drying has been completed by employing a suitable vacuum step.

In the accompanying drawings, I have illustrated a preferred apparatus, but it is to be understood that this apparatus may be suitably modified in order to carry out the invention 30 within the scope of the appended claims.

In the attached drawing there is shown diagrammatically the apparatus which I employ for processing of wood or wood products with the vapor-liquid method for the production of hydrolyzed wood.

In the drawing A is a horizontal metal retort or cylinder such as, for example, a creosoting cylinder. B is a cylindrical basket-like container for wood shavings, sawdust, chips or similar mechanically disintegrated wood substance. This basket is constructed of wire mesh of suitable size covering a rigid frame work 10. Spiral baffles 11 are arranged within this frame work to aid in mixing the material when the basket is 45 rotated. The numeral 12 indicates an engaging device such as a female gear to accommodate a gear 13 on the shaft 14 which passes through packing gland 15 to the sprocket 16 driven by a chain 17 from motor 18 and serves as a means for slow speed rotation of the basket B. The numeral 19 indicates a bearing on the cylinder B which receives the stationary shaft 20 on the door of the retort. When the door of the retort is closed the shaft 20 and bearing 19 support the cylinder B in cooperation with the rotating supporting means 13 and 14.

Rollers 21 supported on cylinder A, which contact circular tracks or bands 22 forming part of frame work 10 on cylinder B, serve to align and 60 support the basket during rotation. Suitable lever operated rollers (not shown) may also be arranged for shifting to contact longitudinal bands 23 of frame work 10 and thus support basket B for loading or unloading from chamber A.

The cylinder A is connected through ports a, b and c to vapor line LV-1 which connects through valve 24 to evaporator or boiler C. The nipples from the line LV-1 through ports a, b and c are extended into the cylinder about 4" to prevent drain back of condensate in the cylinder to line LV-1. Through ports d, e and f the cylinder is connected to vapor line LV-2 having valves 25 and 26 to line LV-3 leading to dephlegmator D or the cylinder is connected

through line LV-4 having valve 27 to condenser E.

The evaporator C is equipped with heat transfer coils 28 through which any suitable heat transfer medium such as heat transfer oil is circulated. Pump 29 circulates heat transfer oil through the heat absorber 30 through line HL-1 to the coils 28. The oil is discharged from the evaporator into line HL-2 and returns to the pump 29.

The following example is illustrative of the manner of using this apparatus to produce hydrolyzed wood of high lignin content.

Comminuted wood, e. g., wood chips having a thickness of about  $\frac{1}{8}$ " and length in the grain direction of the wood of about  $\frac{1}{4}$ " are loaded into the basket B. The basket is then placed in the cylinder A as shown in the drawing, and the door is closed and bolted. A solution of sulfuric acid, of about 1% strength, is forced from a suitable storage, not shown, through line LL-9 having valve 31 by a pump, not shown, through valve 32, pump 33, and valve 34 to spray line SL-1 and spray header 35; the acid solution being sprayed on the basket and its contents during slow rotation of the basket. When the comminuted wood in the basket has been saturated to the desired extent with acid, as may be determined by gauging the tank from which the acid is being drawn, the pump is stopped and valves 31, 32 and 34 are closed. During the spraying operation any of the acid solution not taken up by the wood may be allowed to drain from the cylinder to tank F by opening valve 36 on line LL-1. It may then be returned to storage by opening valve 37 on line LL-11, by a suitable pumping means, not shown. The cylinder A is then connected to the atmosphere through line LV-2 by opening valves 25 and 27 to condenser E and valve 38 on line LV-5. Steam is then introduced to the cylinder from the evaporator C (which in this case may be a simple steam boiler) by opening valve 35 on line LV-1. As soon as the air in the cylinder has been displaced by the steam, as will be shown by live steam being discharged from line LV-5, valves 25, 27, and 38 are then closed. Valves 39 and 40 are then opened, the steam passing from the evaporator through lines LV-1, LV-2 to the cylinder A. Steam pressure in the cylinder A is thereby rapidly increased to 105-135 lbs./sq. in., which usually requires from 3 to 5 minutes. During this time the basket B is kept rotating at a rate of 5 to 15 R. P. M. Valve 36 is partially opened to allow condensate containing reaction products from the wood to drain into condensate tank F, valve 41 on line LV-8 being opened to condenser E. In this manner condensates from the cylinder A is being continually removed from the hydrolyzing theater and is being concentrated in tank F by the flashing off of steam and steam volatile products to the condenser E which may be operating also as a heat exchanger to recover heat from the steam. In lieu of the manually operated drain valve 36 an automatic condensate discharge trap may be employed to transfer the condensate from the cylinder A to the condensate tank F.

The conditions of temperature (340° F. to 360° F.) and pressure (105 to 135 lbs./sq. in.) are maintained in the cylinder for the necessary time required to give the desired lignin content in the final product. About 20 to 30 minutes under the operating conditions described above will yield a product having a lignin content of 40 to 45%.

At the end of this time valves 39 and 40 are closed and valve 36 is closed after being opened for a short time to assure complete discharge of condensate from the cylinder. Pressure is then released by opening valves 25 and 26 to heat exchanger D, the steam and steam volatile products passing from the cylinder to D through lines LV-2 and LV-3. Wash water, needed later, may be heated by passing it through line LL-2 having valve 42 to the tube section of heat exchanger D, during this pressure releasing operation. The wash water may be circulated from a suitable storage, not shown, by means of a pumping means, not shown, entering the heat exchanger D through line LL-2 and passing through the tube section of D to a suitable discharge line, not shown, returning to the wash water storage.

Condensate forming in D may be allowed to fill that heat exchanger and spill over to condenser E by opening valve 43 on line LV-12.

Condensation of steam and steam distilled by-products from the wood occurs in condenser E when water is introduced to the tube section of that condenser by suitable means, not shown. The condensate is collected in condensate receiving tank H and may be transferred therefrom to a volatile by-product storage or to suitable fractionating equipment, not shown, through line LL-5 having valve 44.

Release of pressure from the cylinder A is usually completed in a matter of from 5 to 10 minutes.

When the pressure in the cylinder A has reached atmospheric, heated wash water at a temperature of 140 to 160° F. is pumped into the cylinder from a suitable source through line LL-9, having valve 31, valves 32 and 34 being opened. The wash water enters the cylinder through spray line SL-1 and spray header 35. By rotating the basket the hydrolyzed wood product is brought into intimate contact with the wash water which serves to accomplish rapid washing of acid and hydrolysis products from the wood. Between washings, which usually require about 30 minutes to 1 hour, the wash water is drained from the cylinder by opening a suitable discharge, not shown, on the bottom of the cylinder. At the end of such periods of draining wash water may be sprayed on the basket and contents and the latter allowed to drain for a short period thereafter before introducing water for the next main washing cycle.

About 3 or 4 such washing cycles will be found sufficient to remove the acid and hydrolysis products, a total of 10 to 15 thousand gallons of wash water per ton of dry hydrolyzed wood, delivered in 3 or 4 washing cycles, are required for the washing.

The damp hydrolyzed product is then vapor dried using the apparatus shown in the attached drawing in accordance with the methods described in my Patent No. 2,273,039 and my application Serial No. 579,851. Operation of the apparatus for drying is the same as that described in the application Serial No. 579,851 except that the wood is contained in a rotating basket instead of on trams which applies in the case of massive wood.

The apparatus shown in the drawing may be used for hydrolysis of wood by vapor treatment with water acidified with small amounts of HCl to prepare it for subsequent treatment with aniline and furfural to produce ligno-cellulose plastic molding powders as described in U. S. Patents

Nos. 1,923,756 and 1,932,255. After hydrolysis the material may be washed in the cylinder B and subsequently dried by introducing vaporized aniline or furfural. Drying by means of aniline or an aldehyde in vapor phase gives a much more thorough and uniform distribution of the plasticizer throughout the mass and the heating of the wood at the boiling point of the chemicals produces a much more stable lignin-cellulose aniline complex, or lignin-cellulose-furfural plastic when the material is molded.

In preparing hydrolyzed products from either massive timber or comminuted wood according to the present invention, where drying is resorted to, this is carried out in accordance with my aforesaid patent and applications to substantially zero moisture content.

The hydrolyzed products obtained, whether from massive timber or comminuted wood, are completely dried and are identifiable because they are substantially devoid of water soluble extracts such as hexose sugars and furfural produced by the hydrolysis action. Moreover the hydrolyzed products are further identifiable by being substantially devoid of organic solvent soluble extractives such as wood gums and resins, either normally present or produced by said hydrolysis because these are removed when the treated wood is completely dried with an organic vapor which is a solvent for such extractives.

To the dried comminuted wood treated as above there may be incorporated a potentially reactive synthetic resin. Among such resins are those obtainable from phenol-aldehyde, amine-aldehyde, urea-aldehyde, Glyptal and cumarone resin components. Preferably about 2% by weight of the potentially reactive synthetic resin is introduced to the comminuted wood which may in some cases be further reduced in size so as to pass through a 20 mesh screen or smaller. In this manner a heat moldable or heat compressible composition is formed.

It will be observed that condensates from the steam and products of the hydrolysis reaction soluble therein are continually removed as formed from contact with the wood and by removing these condensates from the treating chamber and lowering the pressure and temperature conditions surrounding them, for example as in the flash tank F, the usual degradation which occurs when these products are left in the environment of the treating conditions in the chamber A is largely prevented and the by-products are in a much more usable and valuable form.

After the hydrolysis treatment the wood is usually washed with water and in the case of comminuted wood as much water expressed therefrom as possible before the same is introduced to the vapor phase drier. This vapor phase drying with an organic vapor, as set forth in my above mentioned patents, not only produces a completely dry wood but, as mentioned above, removes the organic solvent soluble extractives produced by the hydrolysis, or already present in the wood. These wood gums, although being resinous in nature, are, as a rule, not generally miscible with synthetic resins and hence will deter the latter from readily wetting and penetrating the wood in the most satisfactory manner and furthermore such wood resins are generally hygroscopic in nature although not water soluble and hence are poor binding agents. Therefore it is desirable that these wood gums or resins be removed.

I claim:

1. The process of hydrolyzing wood which comprises treating the wood in a closed chamber with steam in the presence of an acid catalyst and simultaneously with hydrolysis of the wood removing from said chamber the condensate from the steam and products of the hydrolysis reaction soluble therein.
2. The process of hydrolyzing wood which comprises treating the wood in a closed chamber with steam in the presence of an acid catalyst and simultaneously with hydrolysis of the wood removing from said chamber the condensates from the steam and products of the hydrolysis reaction soluble therein, and thereafter removing organic solvent soluble extractives produced by the hydrolysis together with such extractives already present in the wood while drying to zero moisture content with an organic solvent vapor.
3. The process of hydrolyzing wood which comprises treating the same in comminuted condition in a closed chamber with steam in the presence of an acid catalyst and simultaneously with hydrolysis of the wood removing from said chamber the condensates from the steam and products of the hydrolysis reaction soluble therein, washing said hydrolyzed wood with water, and thereafter removing organic solvent soluble extractives produced by the hydrolysis together with such extractives already present in the wood while drying to zero moisture content with an organic solvent vapor.
4. The process of hydrolyzing wood which comprises treating the same in comminuted condition in a closed chamber with steam in the presence of an acid catalyst and simultaneously with hydrolysis of the wood removing from said chamber the condensates from the steam and products of the hydrolysis reaction soluble therein and recovering the said by-products of the hydrolysis continuously as formed during hydrolysis of the wood, washing said hydrolyzed wood with water, and thereafter removing organic solvent soluble extractives produced by the hydrolysis together with such extractives already present in the wood while drying to zero moisture content with an organic solvent vapor.
5. The process of treating wood which comprises wetting the wood with a dilute mineral acid, subjecting the wood in a closed chamber to the action of live steam and simultaneously with said treatment of the wood removing from contact therewith the wood condensates and reaction products of the treatment soluble in said condensates, subjecting the treated wood to washing with water, expressing the water from the washed and treated wood, and drying the washed and treated wood in the presence of an organic drying medium in vapor phase which is a solvent for the organic solvent soluble products produced by the treatment as well as such products already present in the wood.
6. A wood treatment process comprising wetting disintegrated wood particles with a dilute mineral acid, subjecting said wood particles in a closed chamber to the action of live steam, maintaining said steam treatment at a temperature of about 340° F. to 360° F. for a time sufficient to give the desired lignin content in the treated wood, washing the thus treated wood particles with water to remove the water soluble reaction products therefrom, and drying the washed wood particles with heated, inert organic vapor which removes the remaining water and the organic

solvent solubles from the wood and effects thorough drying of the wood.

7. A process of treating wood to render it suitable for resin impregnation, comprising wetting the wood with a dilute solution of a mineral acid, subjecting the wood in a closed chamber to the action of live steam, continually removing the wood condensates and reaction products soluble therein from said chamber so as to avoid degradation thereof, continuing the steam treatment until the desired lignin content in the wood is obtained, washing the thus treated wood with water to remove water solubles, and then drying the washed wood by passing through said chamber a flow of highly heated, inert, organic drying vapor that removes the moisture and the organic solvent solubles from the wood.

8. A process of treating wood to render it suitable for resin impregnation, comprising wetting the wood with a dilute solution of a mineral acid, subjecting the wood in a closed chamber to the action of live steam at a pressure of about 105-135 pounds per square inch, continually removing the wood condensates and reaction products soluble therein from said chamber so as to avoid degradation thereof, maintaining the steam treatment at a temperature of about 340° F. to 360° F. until a lignin content of about 40% to 45% in the wood is obtained, washing the thus treated wood with hot water to remove water solubles, repeating this washing treatment a plurality of times and removing the wash water from the chamber, and then drying the washed wood by passing through the chamber a flow of highly heated,

inert, organic drying vapor that removes the moisture and the organic solvent solubles from the wood.

MONIE S. HUDSON.

#### 5 REFERENCES CITED

The following references are of record in the file of this patent:

#### 10 UNITED STATES PATENTS

|    | Number    | Name             | Date          |
|----|-----------|------------------|---------------|
| 10 | 150,111   | Voelter          | Apr. 21, 1874 |
|    | 1,037,185 | Gallagher et al. | Aug. 27, 1912 |
|    | 1,059,820 | Besenfelden      | Apr. 22, 1913 |
| 15 | 1,087,743 | Ekstrom          | Feb. 17, 1914 |
|    | 1,890,304 | Scholler         | Dec. 6, 1932  |
|    | 2,080,077 | Howard           | May 11, 1937  |
|    | 2,108,567 | Scholler         | Feb. 15, 1938 |
|    | 2,123,211 | Scholler         | July 12, 1938 |
| 20 | 2,123,212 | Scholler         | July 12, 1938 |
|    | 2,153,316 | Sherrard         | Apr. 4, 1939  |
|    | 2,156,160 | Olson            | Apr. 25, 1939 |
|    | 2,196,277 | Schorger         | Apr. 9, 1940  |
| 25 | 2,315,372 | Kressman         | Mar. 30, 1943 |
|    | 2,323,194 | Beveridge        | June 29, 1943 |
|    | 2,325,570 | Katzen           | July 27, 1943 |

#### FOREIGN PATENTS

|    | Number  | Country | Date          |
|----|---------|---------|---------------|
| 30 | 435,896 | Canada  | July 23, 1946 |

#### OTHER REFERENCES

Katzen et al.: Ind. Eng. Chem., pp. 314-322, vol. 34, No. 3 (Mar. 1942).